

## UNITED STATES PATENT OFFICE.

SAMUEL E. SHEPPARD, OF ROCHESTER, NEW YORK, ASSIGNOR TO EASTMAN KODAK COMPANY, OF ROCHESTER, NEW YORK, A CORPORATION OF NEW YORK.

## PHOTOGRAPHIC LIGHT-SENSITIVE MATERIAL AND PROCESS OF MAKING THE SAME.

No Drawing.

Application filed June 6, 1924. Serial No. 718,411.

*To all whom it may concern:*

Be it known that I, SAMUEL E. SHEPPARD, a subject of the King of Great Britain, residing at Rochester, in the county of Monroe and State of New York, have invented certain new and useful Improvements in Photographic Light-Sensitive Materials and Processes of Making the Same, of which the following is a full, clear, and exact specification.

This invention relates to the art of photographic materials.

One object of the invention is to provide photographic emulsions, especially developing-out ones, having new or improved properties because of the use or presence therein of materials, the sensitizing properties of which I have discovered. Still another object of my invention is to provide processes in which such materials are used to improve photographic emulsions, especially developing-out ones, as regards light-sensitivity, by which term I include their ability to give the earliest visible impression or image with the minimum exposure or their ability to give density after a given exposure or both, the usual photographic fluid treatments being used in preparing such impression or image or density.

A further object of the invention is to provide colloid products, such for instance as gelatins, the usefulness of which for forming light sensitive photographic emulsions, especially developing-out emulsions, is greatly increased and controlled by my said sensitizing materials incorporated therewith. Another object of the invention is to provide processes for preparing said colloid products or intermediates.

Other objects are,—to increase the sensitivity of photographic emulsions, especially developing-out emulsions, while wholly or partially dispensing with expensive or long and uncertain so-called ripening methods; to enable the use of a type of gelatin having desirable physical qualities in making such a photographic emulsion of greater light-sensitivity than that normally obtainable with said gelatin; to obtain more stable emulsions through the purity of the ingredients; to increase the light-sensitivity of photographic emulsions, particularly developing-out ones, the grain characteristics of which have already been determined; to increase the general light-sensi-

tiveness of such photographic emulsions throughout the spectral ranges to which they are normally sensitive; to make such photographic emulsions of standard light-sensitive characteristics with gelatins which normally do not produce emulsions having such characteristics; to make, as intermediates in the manufacture of photographic emulsions, gelatins of standard light-sensitivity giving power out of gelatins which do not normally have the power of giving such standard sensitivity to emulsions, such as developing-out ones, made from them. Further objects will hereinafter appear.

I have found that certain related series of chemical compounds produce remarkable light-sensitizing effects upon photographic emulsions, especially developing-out ones, when incorporated therein. Broadly speaking each compound of these series contains a divalent atom of the sulfur group (a sulfur atom in one series, a selenium atom in another series, a tellurium atom in still another series) which is joined by a double bond to a single metalloid atom (not one bond to one atom, and the other bond to a different atom) to which at least another group of atoms is attached. Generally it is desirable that the last mentioned group of atoms be such that it induces in the compound a chemical affinity for silver halids,—for instance the compound may combine to an appreciable extent with silver halid to form a soluble complex salt, when said atomic group is present. Moreover, the metalloid atom to which the atom of sulfur, selenium, or tellurium is joined by a double bond is in many instances, but not necessarily, a carbon atom.

For some of the preferred examples of my invention, I select from the above series the following subseries,—thiocarbamids, selenocarbamids, and tellurocarbamids. As the corresponding carbamids are likewise usable in preferred examples of my invention and are readily changed into said carbamids, especially for instance in emulsions of the alkaline or ammonia type, it will be understood that the corresponding carbamids are included hereinafter when said carbamids are claimed. These subseries of carbamids and carbimids include many compounds containing one or more substituent radicals, such as alkyl, aryl, acyl, alkyloxy, aryl-oxy, etc., groups. Thus, for example, allylthi-

ourea (thiosinamine) containing an allyl radical in place of one of the hydrogen atoms of thiourea, is especially useful in practicing my invention. So are allyl isothiocyanate, 5 allyl isoselenocyanate, allyl selenourea, and the corresponding tellurium compounds. Not only can each compound of my series of light-sensitizers be used alone to improve an emulsion (or colloid for an emulsion) but 10 two or more of such compounds may be used together to obtain their mutual or cumulative effects.

It is a common characteristic of the compounds which I use, that said double bonded 15 atom of the sulphur group is chemically held in the molecule with intermediate firmness. Such atom does not react on silver halids as readily as the sulphur atom in sodium sulphide for instance, but it separates out more 20 readily than the sulphur atom in ethyl mercaptan for example. Consequently said double bonded sulphur-group atoms in my compounds correspond roughly in the firmness with which they are held to the firmness 25 with which the sulphur atoms are held in the so-called potential mercaptans, although there is, of course, some range of difference in the firmness with which said double-bonded atoms are held in the different com- 30 pounds of my series. The sensitiveness of the grains of silver halid in emulsions has been shown to correspond to the presence in said grains of nuclei of unstated chemical composition. I, therefore, attribute the sen- 35 sitizing action of my compounds to their forming in the emulsion grains small, mostly ultramicroscopic, nuclei which includes silver combined with either sulfur, or selenium, or tellurium, such as silver sulfid, 40 silver selenid, and silver tellurid. The intermediate firmness with which said double-bonded atoms are held in my compounds facilitates this scattered formation or reaction without reacting on the whole of each 45 grain. Since this deduction is not indispensable to the practical using of my invention, I do not wish to be limited to it except as defined in the claims.

I have also found that the proportions in 50 which my compounds are incorporated in the emulsions (or in the colloids for the emulsions) are important. If used in too high concentrations, they cause fog, and sometimes reversal. The largest proportions 55 which can be effectively used vary somewhat with the particular sensitizing compound or compounds which are used, with the proportion of gelatin to silver halid in the emulsion, with the type of emulsion as re- 60 gards grain size characteristics and alkalinity with the amount of natural sensitizer originating in the gelatin when the latter is manufactured, with the particular silver halid or halids employed, the standard as 65 regards fog which is set by the emulsion

maker, etc. This maximum proportion is in any specific case easily found, being about as readily determined by routine test as, for example, the proportion of sulfur permissible in steel for a particular purpose. It is, 70 however, always surprisingly small. In general with gelatino-silver-halid developing-out emulsions, it should be less than about 10 grains of active sensitizing compound, such as thiosinamine for example, in 130 75 pounds of emulsion (the latter being computed as the weight of its non-aqueous ingredients in the dry state); or less than about 10 grains in 100 pounds of gelatin (computed as dry gelatin), when it is added 80 to the gelatin before the latter is used in making the emulsion. A quantity which causes immediate fogging tendency should not to be used,—that is, a quantity which causes more than the tolerated fog allowed 85 in the particular type of emulsion in the trade after the customary allowed period of storage. I have found 2 to 3 grains of sensitizing compound, such as thiosinamine for instance, to 100 pounds of 90 gelatin (computed as dry) or 130 pounds of emulsion (computed as dry) is within the useful limits and generally excellent,—say for instance with alkaline developing-out 95 gelatino-silver-halid emulsions. Of course, smaller amounts of sensitizers are employed when less sensitizing effects are desired; but it is important not to exceed the upper limits as stated above.

Because only very minute quantites of 100 my sensitizing compounds are used, (often less than one three hundred thousandth of the weight of emulsion) the addition of them does not appreciably dilute the emulsion or 105 emulsion-forming colloid; nor does it affect their physical properties. Consequently the use of my compounds provides a novel, dependable and independent way for controlling the properties of photographic emulsions in addition to the customary expedients hitherto available. Gelatins, for 110 instance, can be selected for their physical properties, such as setting ability, melting point and viscosity, without regard to 115 whether they can be made into sufficiently light-sensitive emulsions, and any deficiency in sensitizing power can be made up by incorporating a little quantity of one or more of my independent compounds. Nor are the grain-size characteristics affected by such additions of my compounds, they being independently controlled by the emulsion maker. In other words, I can establish a ratio of sensitizing compounds to silver halid in the emulsions which is independent of the ratio of gelatin to silver halid. Still differently stated, the sensitizer compounds can be added without adding any colloid, such as gelatin, and are, therefore, independent thereof.

My sensitizing compounds act as so-called "chemical" sensitizers instead of as "optical" sensitizers. In other words, they increase the "general" sensitiveness of photographic emulsions, notably developing-out ones, in which they are incorporated,—that is to light of substantially the same wave lengths as those to which the emulsion would be sensitive without the incorporation of my compounds; instead of merely increasing the sensitiveness to some narrow group of wave lengths. Unlike the effects of dyes, the sensitiveness is increased throughout the normal spectral range of the emulsion instead of at only those spectral points corresponding to the spectral absorption of the sensitizing compound. My compounds are effective in increasing the general light-sensitiveness of orthochromatic, panchromatic, X-ray, and all special emulsions, as well as the ordinary or non-color-sensitized ones. They can be added without or with sensitizing dyes or before or after them. They do not specifically affect the dye action; but simply increase the general sensitiveness and thus increase the ordinary sensitiveness to blue light to at least as great an extent as to light of a color corresponding to the dye.

My sensitizing compounds may be used in many ways. Broadly they may be incorporated in emulsions or in colloids for emulsions or both. They can also enter the emulsion mixed with other ingredients thereof whether organic or inorganic. They may be added at different stages of emulsion manufacture, even when the latter is otherwise complete ready for coating. Since their action is rapid when incorporated, the coating in such case need be delayed only long enough to mix in the sensitizing compounds. With the grain characteristics, such as size distribution, etc., already determined, and the other physical and photographic properties of the emulsion already taken care of at this stage, I can practically independently increase its light-sensitivity without impairing said other properties by adding one or more of my compounds. The latter are especially effective in emulsions which are, at least slightly, alkaline.

Where different batches of emulsion, especially developing-out emulsions, fall below a required manufacturing standard of light sensitiveness, although they may be otherwise satisfactory, their sensitiveness can readily be brought up to standard by mixing in my sensitizing compounds, the proportion varying with the increase necessary to produce a uniform product. Emulsions having almost no practical light sensitiveness but having enough other desirable qualities can be made usefully light-sensitive by my compounds. Thus the latter are useful in connection with emulsions having good initial light-sensitivity and those

having almost no initial sensitiveness. The increase in sensitiveness can be effected in one step by thoroughly stirring all of the sensitizing compound into the emulsion at one time; or it may be incorporated part at a time in successive steps. When making new batches of emulsion from the same materials which have yielded deficient emulsions, correctional quantities of my sensitizing compounds can be premixed with an ingredient, such as gelatin.

The following example illustrates how light-sensitive photographic emulsions of the developing-out type may be prepared and improved by the aid of one or more of my sensitizing compounds. Of course, my invention is not restricted to this illustration, except as indicated in the claims. The emulsion-forming operations hereinafter described are along the lines of known practice, see for instance "Die Photographie mit Bromsilber Gelatin" by J. M. Eder, published in Halle, Germany in 1903 by Wilhelm Knapp as Part III of Eder's "Auszählliches Handbuch der Photographie."

The two following solutions are made up, the parts being by weight:

|     |                                    |    |
|-----|------------------------------------|----|
| A { | 900 parts of silver nitrate in     | 95 |
|     | 9,200 parts of water.              |    |
| B { | 690 parts of potassium bromide and |    |
|     | 50 parts of potassium iodide in    |    |
|     | 6,100 parts of water along with    |    |
|     | 300 parts of gelatin.              |    |

In mixing B, the halid salts are first dissolved, the water and the gelatin then added to the salt solution. Solution B is then warmed, say to 140° F. or 150° F. for example; and the silver nitrate solution A is gradually added to it with constant stirring. It is preferable to warm solution A before adding it to B, say to 150° F. or 160° F. for instance. When solution A has been thoroughly incorporated in solution B, there are then added 43 parts of strong ammonia previously dissolved in 900 parts of water. The emulsion formed by these operations is allowed to stand for a short time, say 15 minutes to a half hour for example. Then 1050 parts of gelatin are dissolved in it with thorough mixing. The emulsion is next cooled, such as by keeping in a cool space, until it sets to a firm jelly. The latter is broken up, as by shredding for instance, and thoroughly washed to remove soluble salts, such as potassium nitrate and any excess potassium halids. The wash water is, of course, cool enough not to melt the pieces of emulsion jelly. The washed emulsion is next remelted to 100° F. and 1050 parts of water soaked. gelatin are thoroughly mixed into it, the temperature then being raised, say between 120° F. and 150° F., for instance, for a short time, say a few minutes. It is then cooled and set. It is an example of the am-

monia or alkaline type of developing-out emulsion.

My sensitizing compounds may be usefully incorporated at any stage of the above described process of preparing the emulsion, even being premixed with solutions A or B with ammonia or with the gelatin, at the initial stages. When the compounds are incorporated in either a partly or wholly prepared emulsion, they are most conveniently handled by dissolving them in a solvent which is inert with respect to the emulsion and simply acts as a vehicle to help in spreading the compounds throughout the emulsion. So long as an even distribution of the compounds throughout the emulsion is effected and the correct proportion of them is added, their particular concentration in the solvent or vehicle is not important. It is good practice to keep the volume of the solution added to the emulsion under 2% of the volume of the emulsion; but this is not indispensable. For example, where 1 part of thiosinamine by weight is to be incorporated into 300,000 parts by weight of the above described emulsion (computed as the weight of its non-aqueous ingredients) the emulsion is melted, the thiosinamine dissolved in ethyl alcohol or water or a mixture of them, the volume of said solvent being under approximately 1.5% of the volume of the melted emulsion, and then the solution is thoroughly mixed into the emulsion. When necessary to minimize dilution, the volume of solution can be kept even below a fraction of 1%.

As indicated hereinabove, my several series include a large number of useful compounds. Illustrative examples, in addition to thiosinamine (allyl thiourea) already mentioned, are: allyl isothiocyanate, phenyl isothiocyanate, phenyl thiourea, thiocarbamide, thiourea, thiosemicarbazide, sodium thiosulfate, (but not sulfate or sulfite) di-o-tolyl thiourea, seleno-mustard-oil (allyl isoselenocyanate), potassium selenocyanide, allyl selenourea, thioacetamid, thioformamid, thiobarbituric acid, telluro-mustard-oil (allyl isotellurocyanate) potassium tellurocyanide, allyl tellurourea. It is preferable to use these compounds in substantially pure or "C. P." form; but impurities which are harmless to the emulsion and are not bulky, can be tolerated. The selenocyanide and tellurocyanide are used in higher proportions than the other listed compounds.

With its light-sensitiveness increased by my compounds, the emulsion, being melted to the desired flowability, is coated on its support, such as glass, film, paper, etc., in the well known way. It is convenient to control and check the process by coating samples of the emulsion before and after the addition of my sensitizing compounds, the coated specimens being tried out photo-

graphically by any well known sensitometric test, or even by comparative camera exposures on the same subject under like conditions. Of course, the usual precautions are observed during the emulsion making and coating processes, such as the use of non-actinic or "safe" light, cleanliness of vessels and air, etc.

The different gelatines sold for photographic emulsion-making may be used in the example given above, hard ones being very useful. The temperatures given are, of course, adjusted if the particular gelatin employed has physical properties, such as melting and setting points, which deviate considerably from the usual ones, such adjustment being a matter of routine control.

Instead, however, of using gelatines which give emulsions of useful but lower sensitiveness even before the addition of my sensitizing material, an almost inert gelatin may be employed,—one which forms an emulsion which produces a developable image, if at all, only after impractically long exposures, and then does not yield an image of desirable density. A gelatin which forms such a practically inert emulsion may be prepared in the way described under the heading "Preparation of ash-free gelatin" in pages 1856 and 1859 of the "Journal of the American Chemical Society", September, 1922, Vol. XLIV, No. 9, being part of an article by Sheppard, Sweet, and Benedict on "Elasticity of purified gelatin jellies as a function of hydrogen-ion concentration." 100

Emulsions of impractically low light-sensitiveness made by the above described process from such prepared gelatin, are transformed by my sensitizing compounds into emulsions which give developable images of excellent density after usefully brief exposures. I have, for example, been able to increase the light-sensitiveness of some such low sensitive emulsions ten or even over twenty times, the exposures for a given subject in the latter case being cut to less than one twentieth of the original one and the image density being made excellent by a corresponding gain. Increases of the same general order of magnitude are made when my sensitizing compounds are added in similar proportions to emulsions which are made from normal photographic gelatins or mixtures of such normal gelatins with said almost inert gelatins, and already have useful, but lower initial sensitiveness. Different percentages of sensitizer produce correspondingly different increases. The increases in developing-out emulsions appear upon the usual developing operations. Customary pyro and metol-hydrochinon alkaline developers are suitable for example. An inert emulsion prepared as above described is a very useful medium or standard in which to test the sensitizing properties of different com-

105  
110  
115  
120  
125  
130

pounds, a sample containing the compound under test being tried out photographically along with a parallel sample of unsensitized emulsion.

5 Instead of the inert gelatin prepared according to the reference given in the preceding paragraph, I can prepare inert gelatins by treating active photographic gelatins with oxidizing agents. The latter oxidize 10 the sulfur in the sensitizing substituted (allyl) thiocarbamide or corresponding carbimide, which occurs naturally in photographic gelatins, thus converting it to a non-sensitizing compound and leaving the gelatins 15 practically inert. Dilute aqueous solutions of a peroxide, such as sodium peroxide (say from 5 to 10% by weight) is intimately mixed into the gelatin and then washed out when the oxidation has occurred. The inert 20 gelatin referred to in the preceding paragraph can be thus oxidized to make its inertness doubly sure.

When preparing inert gelatin on a considerable scale, it is far preferable to introduce 25 the oxidizing step during the regular manufacturing operations, say the liming and/or deliming treatments. The oxidizing agents should be effective as desensitizers and yet not be present in quantities capable 30 of materially reducing the yield of gelatin or harming its quality, especially its physical properties. Nor should they leave objectionable products from the oxidation reaction. For example, the regular liming 35 solution of the usual gelatin manufacturing process can be saturated with as much calcium hypochlorite as will dissolve therein; or it can contain about 5 to 10% of sodium peroxide. Subsequent operations then proceed 40 as usual.

My sensitizing compounds may be incorporated into gelatin from which photographic emulsions are to be made. This "strengthened" gelatin then constitutes a 45 valuable "intermediate" in emulsion manufacture. While any good gelatin may be thus treated, that which has been rendered inert by the above described oxidation treatment during liming or deliming is particularly 50 adapted to this strengthening. Emulsions made from the mixture have markedly increased light-sensitiveness as compared with those made from corresponding un-strengthened gelatins. The proportion of 55 sensitizing material is, of course, adjusted to give the desired control of the sensitiveness of emulsions made from the gelatin, the total sensitizing material in the "strengthened" gelatin being thus brought to, or even 60 above, normal.

When working on a considerable scale, this activating of gelatin, such, for instance, as said inert gelatin, is one of the most desirable ways of employing my sensitizing

compounds. In fact, premixing of one or 65 more of my sensitizers with gelatin is my preferred system. During manufacture of the gelatin, say for instance when the concentrated gelatin solution comes from the evaporator before setting and drying, the 70 sensitizing compound or compounds are added and thoroughly mixed to obtain effectively uniform distribution. For example 75 2 or 3 grains of thiosinamine or any of the hereinabove listed compounds or mixtures of them is carefully mixed with each fraction of gelatin solution containing 100 pounds of gelatin (calculated as dry). The compound, say thiosinamine, is taken up, 80 preferably in as little aqueous-alcohol mixture as is practicable, and then this concentrated solution added to the gelatin solution. In this way undesirable dilution of the latter is avoided.

On a large scale, the sensitizing solution 85 may be accurately and continually dosed into a regulated stream of gelatin solution with continuous mixing. Alternatively dried or set gelatin may be allowed to swell in an aqueous solution of the sensitizing compound. The nearly uniform distribution or diffusion of the compound in the gelatin thus effected can be made even more nearly uniform by melting and agitating the swollen 90 gelatin.

In the examples given above, the steps 95 of treating with ammonia and warming of the emulsion just before its final setting improve the photographic properties of the emulsion, especially when the latter is made 100 from hard gelatins. But one or both of them may be omitted. In other words, my sensitizing compounds act by themselves to increase the light-sensitiveness, whether ripening steps be employed or not, and so can 105 wholly or partially replace them. But I prefer to use them because the effect of either or both of them is to help increase the light-sensitiveness of the emulsions and thus give a stronger initial sensitized condition 110 which is multiplied or increased by using my sensitizing compounds. When using any of the inert gelatins mentioned above in making very sensitive emulsions, these steps can sometimes be shortened and made 115 more certain in effect by reason of the use of my powerful and dependable sensitizing compounds.

I have described gelatin emulsions and emphasized the developing-out and alkaline 120 types because at the present time they are the ones which have the widest practical use. Moreover they form the best medium for testing new sensitizing-compounds. But other organic colloids and mixtures of them 125 with each other or with gelatin, where their nature admits such mixtures, may be used in making light-sensitive emulsions which

can be improved by adding my sensitizing material. Albumens, agar-agar, gums, such as gum-arabic, cellulosic derivatives such as collodion are instanced. While I have illustrated the use of my sensitizer in connection with such sensitive substances as silver bromide and silver iodide, other light-sensitive substances can be employed, such as silver chlorid, alone or mixed with one or more of the others.

Having thus described my invention, what I claim as new and desire to secure by Letters Patent is:

1. A photographic emulsion comprising a colloid, particles of photographic silver salt suspended therein, and an added compound therein upon which at least part of the light-sensitivity of the emulsion depends, said compound containing a divalent atom of the sulfur group directly joined by a double bond to a single metalloid atom, to which at least another group of atoms is attached, the proportion of said compound being substantially independent of the proportion of said colloid.

2. A photographic developing-out emulsion comprising a colloid, particles of silver halid suspended therein, and an added compound therein upon which at least part of the light-sensitivity of the emulsion depends, said compound having a chemical affinity for silver halid and containing an atom of the sulfur group joined to a single metalloid atom, to which at least another group of atoms is attached, the presence of said last named group inducing said chemical affinity, the proportion of said compound being substantially independent of the proportion of said colloid.

3. A photographic developing-out emulsion comprising gelatin, particles of silver halid suspended therein, and an added compound therein upon which at least part of the light-sensitivity of the emulsion depends, said compound containing a divalent atom of the sulfur group directly joined by a double bond to a single carbon atom to which at least another group of atoms is attached, the proportion of said compound being substantially independent of the proportion of said gelatin.

4. A photographic developing-out emulsion comprising a colloid, particles of photographic silver salts suspended therein, an added compound which forms small ultra-microscopic nuclei of a silver compound containing an atom of the sulfur group, said nuclei being located on said particles of silver halid, the proportion of said compound being substantially independent of the proportion of said colloid.

5. A photographic developing-out emulsion comprising gelatin, particles of silver halid suspended therein, and an added sen-

sitizer containing thiocarbamid upon which at least part of the light sensitivity of the emulsion depends, the proportion of said thiocarbamid being substantially independent of the proportion of gelatin.

6. A photographic developing-out emulsion comprising gelatin, particles of photographic silver salt suspended therein and thiosinamine added therein upon which at least part of the light-sensitivity of the emulsion depends, the proportion of said thiosinamine being substantially independent of the proportion of said gelatin.

7. A photographic developing-out gelatino-silver-halid emulsion of the alkaline type of relatively high light-sensitivity, comprising a mixture of the constituents of a gelatino-silver-halid emulsion of lower light-sensitivity, and an added sensitizing compound upon which depends the difference between said lower and said high light-sensitivity, said compound containing a divalent atom of the sulfur group directly joined by a double bond to a single metalloid atom to which at least another group of atoms is attached, the proportion of said compound being substantially independent of the proportion of gelatin.

8. A photographic developing-out gelatino-silver-halid emulsion of the alkaline type of relatively high light-sensitivity, comprising a mixture of the constituents of a gelatin-silver-halid emulsion of lower light-sensitivity and an added sensitizing compound upon which depends the difference between said lower and said high light-sensitivity, said compound having a chemical affinity for silver halid and containing an atom of the sulfur group joined to a single metalloid atom to which at least another group of atoms is attached, the presence of said last named group inducing said chemical affinity, and the proportion of said compound being substantially independent of the proportion of said colloid.

9. A photographic developing-out gelatino-silver-halid emulsion of the alkaline type of relatively high light-sensitivity, comprising a mixture of the constituents of a gelatino-silver-halid emulsion of lower light-sensitivity and an added sensitizing compound upon which depends the difference between said lower and said high light-sensitivity, said compound containing a divalent atom of the sulfur group directly joined by a double bond to a single carbon atom to which at least another group of atoms is attached, the proportion of said compound being substantially independent of the proportion of the gelatin.

10. A photographic developing-out gelatino-silver-halid emulsion of the alkaline type of relatively high light-sensitivity, comprising a mixture of the constituents of

- a gelatino-silver-halid emulsion of lower light-sensitiveness and a sensitizer comprising thiocarbamid upon which depends the difference between said lower and said high 5 light-sensitiveness, the proportion of sensitizer being substantially independent of the proportion of gelatin.
11. A photographic developing-out gelatino-silver-halid emulsion of the alkaline 10 type of relatively high light-sensitiveness, comprising a mixture of the constituents of a gelatino-silver-halid emulsion of lower light-sensitiveness and a sensitizer comprising thiosinamine upon which depends the 15 difference between said lower and said high light-sensitiveness, the proportion of said sensitizer being substantially independent of the proportion of gelatin.
12. A photographic emulsion comprising 20 a colloid, particles of photographic silver salt suspended therein and an added compound therein upon which at least part of the light-sensitiveness of the emulsion depends, said compound containing a divalent 25 atom of the sulfur group directly joined by a double bond to a single metalloid atom to which at least another group of atoms is attached, said emulsion being free from sensitizing dye, and the proportion of said compound being substantially independent of 30 the proportion of said colloid.
13. A photographic emulsion comprising gelatin, particles of silver halid suspended 35 therein and an added compound therein upon which at least part of the light-sensitiveness of the emulsion depends, said compound having a chemical affinity for silver halid and containing an atom of the sulfur group joined to a single metalloid 40 atom to which at least another group of atoms is attached, the presence of said last named group inducing said chemical affinity, said emulsion being substantially free from sensitizing dye, and the proportion of said compound being substantially independent 45 of the proportion of said gelatin.
14. A photographic emulsion comprising gelatin, particles of silver halid suspended 50 therein and an added compound therein upon which at least part of the light-sensitiveness of the emulsion depends, said compound containing a divalent atom of the sulfur group directly joined by a double bond to a single carbon atom to which at 55 least another group of atoms is attached, the proportion of said compound being substantially independent of the proportion of gelatin, said emulsion being substantially free from sensitizing dye.
15. A photographic developing-out emulsion comprising gelatin, particles of silver halid suspended therein and an added sensitizer containing thiocarbamid upon which at least part of the light-sensitiveness of the 60 emulsion depends, said emulsion being substantially free from sensitizing dye, and the proportion of said compound being substantially independent of the proportion of said gelatin.
16. A photographic emulsion comprising 70 gelatin, particles of silver halid suspended therein and an added thiosinamine upon which at least part of the light-sensitiveness of the emulsion depends, said emulsion being substantially free from sensitizing dye, 75 and the proportion of thiosinamine being substantially independent of the proportion of gelatin.
17. A photographic emulsion comprising 80 a colloid, particles of photographic silver salt suspended therein and an added compound therein upon which at least part of the light-sensitiveness of the emulsion depends, said compound containing a divalent atom of the sulfur group directly joined by 85 a double bond to a single metalloid atom, to which at least another group of atoms is attached, the amount of added compound being less than the order of 10 grains per 130 pounds of emulsion and insufficient to 90 cause immediate fogging tendency.
18. A photographic developing-out emulsion comprising a colloid, particles of silver halid suspended therein, and an added compound therein upon which at least part of 95 the light-sensitiveness of the emulsion depends, said compound having a chemical affinity for silver halid and containing an atom of the sulfur group joined to a single metalloid atom to which at least another group of atoms is attached, the presence of said last named group inducing said chemical affinity, the amount of added compound being less than the order of 10 grains per 130 pounds of emulsion and insufficient to cause 100 immediate fogging tendency.
19. A photographic developing-out emulsion comprising gelatin, particles of silver halid suspended therein, and an added compound therein upon which at least part of 105 the light-sensitiveness of the emulsion depends, said compound containing a divalent atom of the sulfur group directly joined by a double bond to a single carbon atom to which at least another group of atoms is attached, the amount of added compound being less than the order of 10 grains per 130 pounds of emulsion and insufficient to cause 110 immediate fogging tendency.
20. A photographic developing-out emulsion comprising gelatin, particles of silver halid suspended therein, and an added sensitizer containing thiocarbamid upon which at least part of the light-sensitiveness of the emulsion depends, the amount of added compound being less than the order of 10 grains per 130 pounds of emulsion and insufficient to cause 115 immediate fogging tendency.
21. A photographic developing-out emulsion comprising gelatin, particles of photo- 120
- 125
- 130

graphic silver salt suspended therein and thiosinamine added therein upon which at least part of the light-sensitiveness of the emulsion depends, the amount of added compound being less than the order of 10 grains per 130 pounds of emulsion and insufficient to cause immediate fogging tendency.

22. A photographic developing-out emulsion comprising a colloid, particles of photographic silver salt suspended therein and an added compound therein upon which at least part of the light-sensitiveness of the emulsion depends, said compound containing a divalent atom of the sulfur group directly joined by a double bond to a single metalloid atom to which at least another group of atoms is attached, the amount of said compound being insufficient to cause fog of greater density than the set tolerance.

23. A photographic developing-out emulsion comprising gelatin, particles of silver halid suspended therein and an added thiocarbamid upon which at least part of the light-sensitiveness of the emulsion depends, the amount of said thiocarbamid being insufficient to cause fog of greater density than the set tolerance.

24. A photographic developing-out emulsion comprising gelatin, particles of silver halid suspended therein and an added thiosinamine upon which at least part of the light-sensitiveness of the emulsion depends, the amount of said thiosinamine being insufficient to cause fog of greater density than the set tolerance.

25. In the process of preparing a developing-out colloid-sensitive-silver-salt emulsion, increasing the light-sensitiveness thereof by incorporating with the other constituents thereof an independent sensitizing compound, said compound containing a divalent atom of the sulfur group directly joined by a double bond to a single metalloid atom to which at least another group of atoms is attached.

26. In the process of preparing a developing-out-colloid-sensitive-silver-halid emulsion, increasing the light-sensitiveness thereof by incorporating with the other constituents thereof an indedpendent sensitizing compound which has a chemical affinity for silver halid and contains an atom of the sulfur group joined to a single metalloid atom to which at least another group of atoms is attached, the presence of said last named group inducing said chemical affinity.

27. In the process of preparing a developing-out gelatino-silver-halid emulsion increasing the light-sensitiveness thereof by incorporating with the other constituents thereof an independent sensitizing compound containing a divalent atom of the sulfur group directly joined by a double bond to a single carbon atom to which at least another group of atoms is attached.

28. In the process of preparing a developing-out gelatino-silver-halid emulsion, increasing the light-sensitiveness thereof by incorporating with the other constituents thereof an independent thiocarbamid.

29. In the process of preparing a developing-out gelatino-silver-halid emulsion, increasing the light-sensitiveness thereof by incorporating independent thiosinamine with the other constituents thereof.

30. In the process of preparing a developing-out colloid-silver-salt emulsion of the alkaline type of relatively high light sensitiveness, combining constituents of a colloid-sensitive-silver-salt emulsion of lower light sensitiveness with sufficient independent sensitizing compound to effect high light sensitiveness, said compound containing a divalent atom of the sulfur group directly joined by a double bond to a single metalloid atom to which at least another group of atoms is attached.

31. In the process of preparing a developing-out gelatino-silver-halid emulsion of the alkaline type of relatively high-light-sensitiveness, combining constituents of a gelatino-silver-halid emulsion of lower light sensitiveness with sufficient independent sensitizing compound to effect said high-sensitiveness, said compound having a chemical affinity for silver halid and containing an atom of the sulfur group joined to a single metalloid atom to which at least another group of atoms is attached, the presence of said last named group inducing said chemical affinity.

32. In the process of preparing a developing-out gelatino silver halid emulsion of the alkaline type of relatively high-light-sensitiveness, combining constituents of a gelatino-silver-halid emulsion of said type but of lower sensitiveness with an independent sensitizing compound to effect said light-sensitiveness, said compound containing a divalent atom of the sulfur group directly joined by a double bond to a single carbon atom to which at least another group of atoms is attached.

33. In the process of preparing a developing-out gelatino-silver-halid emulsion of the alkaline type of relatively high light sensitiveness, combining constituents of a gelantino-silver-halid emulsion of said type but of lower light-sensitiveness with an independent thiocarbamid to effect said high light-sensitiveness.

34. In the process of preparing a developing-out gelatino-silver-halid emulsion of the alkaline type of relatively high light-sensitiveness, combining constituents of a gelatino-silver-halid emulsion of said type of lower light-sensitiveness with an independent thiosinamine to effect said high light-sensitivity.

35. In the process of preparing a develop-

70

75

80

85

90

95

100

105

110

115

120

125

130

ing-out gelatino-silver-salt emulsion, increasing the light-sensitiveness thereof by incorporating with the other constituents thereof, which are free from sensitizing dye, 5 an independent sensitizing compound, which is free from sensitizing dye, containing a divalent atom of the sulfur group directly joined by a double bond to a single metalloid atom to which at least another group 10 of atoms is attached.

36. In the process of preparing a developing-out colloid-sensitive-silver-salt emulsion, increasing the light-sensitiveness thereof by incorporating with the other constituents 15 thereof, which are substantially free from sensitizing dye, an independent sensitizing compound which is substantially free from sensitizing dye, said compound having a chemical affinity for silver halid and containing an atom of the sulfur group joined to a single metalloid atom to which at least another group of atoms is attached, the presence of said last named group inducing said chemical affinity.

37. In the process of preparing a developing-out colloid-sensitive-silver-salt emulsion, increasing the light-sensitiveness thereof by incorporating with the other constituents thereof, which are substantially free from 25 sensitizing dyes, an independent sensitizing compound, which is also substantially free from sensitizing dye, said compound containing a divalent atom of the sulfur group directly joined by a double bond to a single 30 carbon atom to which at least another group of atoms is attached.

38. In the process of preparing a developing-out gelatino-silver-halid emulsion, increasing the light-sensitiveness thereof by incorporating with the other constituents 40 thereof, which are substantially free from sensitizing dye, an independent thiocarbamid substantially free from sensitizing dye.

39. In the process of preparing a developing-out colloid-sensitive-silver salt emulsion, increasing the light-sensitiveness thereof by incorporating with the other constituents thereof, which are substantially free from sensitizing dye, an independent thiosinamine 45 substantially free from sensitizing dye.

40. In the process of preparing a developing-out colloid-sensitive-silver-salt emulsion, increasing the light-sensitiveness thereof by incorporating with the other constituents 55 thereof an independent sensitizing compound containing a divalent atom of the sulfur group directly joined by a double bond to a single metalloid atom to which at least another group of atoms is attached, the amount of said added compound being less than the order of 10 grains per 130 pounds of emulsion and being insufficient to cause immediate fogging tendency.

41. In the process of preparing a develop-

ing-out colloid-sensitive-silver-salt emulsion, increasing the light-sensitiveness thereof by incorporating with the other constituents thereof an independent sensitizing compound, said compound containing a divalent atom of the sulfur group directly 65 joined by a double bond to a single metalloid atom to which at least another group of atoms is attached, the amount of said added compound being less than the order of 10 grains per 130 pounds of emulsion 70 and insufficient to cause immediate fogging tendency.

42. In the process of preparing a developing-out colloid-sensitive-silver-halid emulsion, increasing the light-sensitiveness thereof by incorporating with the other constituents thereof an independent sensitizing compound which has a chemical affinity for silver halid and contains an atom of the sulfur group joined to a single metalloid 80 atom to which at least another group of atoms is attached, the presence of said last named group inducing said chemical affinity, the amount of said added compound being less than the order of 10 grains per 130 85 pounds of emulsion and insufficient to cause immediate fogging tendency.

43. In the process of preparing a developing-out gelatino-silver-halid-emulsion, increasing the light-sensitiveness thereof by incorporating with the other constituents thereof an independent sensitizing compound containing a divalent atom of the sulfur group directly joined by a double bond to a single carbon atom to which at 90 least another group of atoms is attached, the amount of said added compound being less than the order of 10 grains per 130 95 pounds of emulsion and insufficient to cause immediate fogging tendency.

44. In the process of preparing a developing-out gelatino-silver-halid emulsion, increasing the light-sensitiveness thereof by incorporating with the other constituents thereof an independent thiocarbamid, the 100 amount of said added compound being less than the order of 10 grains per 130 pounds of emulsion and insufficient to cause fogging tendency.

45. In the process of preparing a developing-out gelatino-silver-halid emulsion, increasing the light-sensitiveness thereof by incorporating an independent thiosinamine with the other constituents thereof, the amount of said added compound being less 110 than the order of 10 grains per 130 pounds of emulsion and insufficient to cause immediate fogging tendency.

46. The process of preparing photographic gelatino-silver-halid emulsions, which 125 comprises substantially freeing gelatin from any sensitizing compounds originating therein, mixing an independent sensitizing

compound therein, and preparing a sensitive photographic emulsion from said mixture.

47. The process which comprises incorporating in a melted developing-out gelatino-silver-halid emulsion an independent sensitizing compound containing a divalent atom of the sulfur group directly joined by a double bond to a single metalloid atom to which at least another group of atoms is attached.

48. In the process of preparing a developing-out gelatino-silver-halid emulsion, mixing with the gelatin an independent sensitizing compound containing a divalent atom of the sulfur group directly joined by a double bond to a single metalloid atom to which at least another group of atoms is attached and thereafter incorporating said mixture with the other ingredients of said emulsion.

49. In the process of making a photographic colloid-sensitive-silver-salt emulsion, incorporating with the other ingredients thereof an added compound upon which at least part of the light-sensitiveness of the emulsion depends, said independent compound containing a divalent atom of the sulfur group directly joined by a double bond to a single metalloid atom to which at least another group of atoms is attached, the amount of said compound being insufficient to cause fog of greater density than the set tolerance.

50. An intermediate for use in making photographic emulsions, comprising an emulsion-forming colloid having incorporated therein an independent sensitizing compound containing a divalent atom of the sulfur group directly joined by a double bond to a single metalloid atom to which at least another group of atoms is attached.

51. An intermediate for use in making photographic emulsions, comprising an emulsion-forming colloid having incorporated therein an independent sensitizing compound, said compound having a chemical affinity for silver halid and containing an atom of the sulfur group joined to a single metalloid atom to which at least another group of atoms is attached, the presence of said last named group inducing said chemical affinity.

52. An intermediate for use in making photographic emulsions, comprising gelatin having incorporated therein an independent sensitizing compound, containing a divalent atom of the sulfur group directly joined to a single carbon atom to which at least another group of atoms is attached.

53. An intermediate for use in making photographic emulsions, comprising gelatin having incorporated therein an independent thiocarbamid.

54. An intermediate for use in making

photographic emulsions, comprising gelatin having incorporated therein independent thiosinamine.

55. An intermediate for use in making photographic emulsions, comprising an emulsion-forming colloid having incorporated therein an independent sensitizing compound containing a divalent atom of the sulfur group directly joined by a double bond to a single metalloid atom to which at least another group of atoms is attached, the amount of said added compound being less than the order of 10 grains in 100 pounds of gelatin.

56. An intermediate for use in making photographic emulsions, comprising an emulsion-forming colloid having incorporated therein an independent sensitizing compound, said compound having a chemical affinity for silver halid and containing an atom of the sulfur group joined to a single metalloid atom to which at least another group of atoms is attached, the presence of said last named group inducing said chemical affinity, the amount of said added compound being less than the order of 10 grains in 100 pounds of gelatin.

57. An intermediate for use in making photographic emulsions, comprising gelatin having incorporated therein an independent sensitizing compound containing a divalent atom of the sulfur group directly joined to a single carbon atom to which at least another group of atoms is attached, the amount of said added compound being less than the order of 10 grains in 100 pounds of gelatin.

58. An intermediate for use in making photographic emulsions, comprising gelatin having incorporated therein an independent thiocarbamid, the amount of said added compound being less than the order of 10 grains in 100 pounds of gelatin.

59. An intermediate for use in making photographic emulsions, comprising gelatin having incorporated therein thiosinamine, the amount of said added compound being less than the order of 10 grains in 100 pounds of gelatin.

60. An intermediate for use in making photographic developing out emulsions, comprising a mixture of gelatin and an independent sensitizing compound containing a divalent atom of the sulfur group directly joined by a double bond to a single metalloid atom to which at least another group of atoms is attached, the proportion of said compound being insufficient to cause fog density exceeding the set tolerance when said intermediate is made into said developing-out emulsions.

61. An intermediate for use in making photographic developing-out emulsions, comprising a mixture of gelatin and an independent thiocarbamid, the proportion of

thiocarbamid being insufficient to cause fog density greater than a set tolerance when said intermediate is made up into said developing-out emulsions.

5 62. An intermediate for use in making photographic developing-out emulsions, comprising gelatin and independent thiosinamine, the amount of thiosinamine being insufficient to cause fog density exceeding the 10 set tolerance when said intermediate is made up into said emulsions.

63. The process of making an intermediate for use in the preparation of photographic emulsions, which comprises incorporating in an emulsion-forming colloid an independent sensitizing compound containing a divalent atom of the sulfur group directly joined by a double bond to a single metalloid atom to which at least another group 20 of atoms is attached.

64. The process of making an intermediate for use in the preparation of photographic emulsions, which comprises incorporating in an emulsion-forming colloid an independent sensitizing compound, said compound having a chemical affinity for silver halid and containing an atom of the sulfur group joined by a single metalloid atom to which at least another group of atoms is attached, the presence of said last named group inducing said chemical affinity.

65. The process of making an intermediate for use in the preparation of photographic emulsions, which comprises incorporating in gelatin an independent sensitizing compound containing a divalent atom of the sulfur group directly joined to a single carbon atom to which at least another group of atoms is attached.

66. The process of making an intermediate for use in the preparation of photographic emulsions, which comprises adding to an emulsion-forming colloid an independent thiocarbamid.

67. The process of making an intermediate for use in the preparation of photographic emulsions, which comprises adding to an emulsion-forming colloid independent thiosinamine.

68. The process of making an intermediate for use in the preparation of photographic emulsions, which comprises incorporating in an emulsion-forming colloid an independent sensitizing compound containing a divalent atom of the sulfur group directly joined by a double bond to a single metalloid atom to which at least another group of atoms is attached, the amount of said added compound being less than the order of 10 grains per 100 pounds of said colloid (calculated as dry colloid) and being insufficient to cause immediate fogging tendency.

69. The process of making an intermediate for use in the preparation of photo-

graphic emulsions, which comprises incorporating in an emulsion-forming colloid an independent sensitizing compound, said compound having a chemical affinity for silver halid and containing an atom of the sulfur group joined by a single metalloid atom to which at least another group of atoms is attached, the presence of said last named group inducing said chemical affinity, the amount of said added compound being less than the order of 10 grains per 100 pounds of said colloid (calculated as dry colloid) and being insufficient to cause immediate fogging tendency. 70

70. The process of making an intermediate for use in the preparation of photographic emulsions, which comprises incorporating in gelatin a sensitizing compound containing a divalent atom of the sulfur group directly joined to a single carbon atom of which at least another group of atoms is attached, the amount of said added compound being less than the order of 10 grains per 100 pounds of said colloid (calculated as dry colloid) and being insufficient to cause immediate fogging tendency. 80

71. The process of making an intermediate for use in the preparation of photographic emulsions, which comprises adding to an emulsion-forming colloid a thiocarbamid, the amount of said added compound being less than the order of 10 grains per 100 pounds of said colloid (calculated as dry colloid) and being insufficient to cause immediate fogging tendency. 90

72. The process of making an intermediate for use in the preparation of photographic emulsions, which comprises adding to an emulsion-forming colloid a thiosinamine, the amount of said added compound being less than the order of 10 grains per 100 pounds of said colloid (calculated as dry colloid) and being insufficient to cause immediate fogging tendency. 100

73. The process of making an intermediate for use in the preparation of photographic emulsions, which comprises incorporating in an emulsion-forming colloid an independent sensitizing compound containing a divalent atom of the sulfur group directly joined by a double bond to a single metalloid atom to which at least another group of atoms is attached, the proportion of said compound being insufficient to cause fogging density greater than the set tolerance. 110

74. The process of making an intermediate for use in the preparation of photographic gelatino-silver-halid emulsions, which comprises substantially freeing gelatin from sensitizing compounds and incorporating therein an independent sensitizing compound. 125

75. The process of making an intermediate for use in the preparation of photographic gelatino-silver-halid emulsions, 130

which comprises substantially freeing gelatin from sensitizing compounds and incorporating therein a sensitizing compound containing a divalent atom of the sulfur group 5 directly joined by a double bond to a single metalloid atom to which at least another group of atoms is attached, the amount of said added compound being less than the or-

der of 10 grains per 100 pounds of said gelatin (calculated as dry gelatin) and being 10 insufficient to cause immediate fogging tendency.

Signed at Rochester, New York, this 4th day of June, 1924.

SAMUEL E. SHEPPARD.